

# United States Patent

[11] 3,613,612

[72] Inventor **Carroll Trowbridge Kennedy**  
Waynesboro, Va.  
[21] Appl. No. **453,478**  
[22] Filed **May 5, 1965**  
[45] Patented **Oct. 19, 1971**  
[73] Assignee **Thiokol Chemical Corporation**  
Bristol, Pa.

[56] **References Cited**  
FOREIGN PATENTS  
635,842 3/1962 Italy ..... 112/43  
*Primary Examiner*—James R. Boler  
*Attorney*—Emil W. Milan

[54] **HIGH-STRENGTH TUFTED PILE FABRIC**  
2 Claims, No Drawings  
[52] U.S. Cl. .... **112/410,**  
161/67  
[51] Int. Cl. .... **D05c 17/02**  
[50] Field of Search. .... **112/410,**  
266, 43; 161/66, 67; 117/139.5 F, 139.5 R

**ABSTRACT:** The invention relates to a high-strength tufted pile fabric having a woven primary backing material of polypropylene or copolymer of propylene yarn, at least some of the yarn having a relatively flat cross section, which has been coated with about 0.2 to 12 percent, based on the weight of the yarn, of a lubricant material prior to penetrating tufts through the bodies of the yarn. The presence of the lubricant material on the yarns of the backing enhances penetration of the tufting needles and tufts into the yarns without the tufting needles causing the otherwise serious rupturing and shattering of the penetrated yarns which occurs during tufting of otherwise similar, but unlubricated, woven primary backing.

## HIGH-STRENGTH TUFTED PILE FABRIC ARTICLES AND METHODS

This invention relates to improved primary backings for tufted pile fabrics, to improved pile fabrics comprising these packings and to methods for producing each.

It is present practice to employ a flat woven burlap-type backing material having yarns composed of jute, sisal, or sometimes paper. A serious disadvantage of this backing resides in the fact that the backing fabric is not of uniform thickness nor density. This characteristic is, of course, due in part to the actual interstices between the individual yarns and in part to the wide variation in thickness between individual yarns and varying thicknesses in the same yarn. As a result, the tufting needles sometimes meet no resistance whatsoever. At the other extreme, the needles encounter maximum resistance due to the necessity for penetrating a thick yarn or double yarns. In still other instances the needles seem to push aside the yarns with little or no penetration of the yarn itself. As a result, the rows of pile yarn stitches frequently jump back and forth between the same longitudinal yarns in the backing thus causing gaps between adjacent rows of stitches which include as few as one and sometimes as many as three yarns of the backing material. This causes grinning and uneven rows of pile. Heretofore it has been found necessary to overcome this disadvantage by producing tufted pile fabrics with sufficient pile length so that these irregularities are substantially concealed. These irregularities occur both longitudinally and transversely of the fabric since a relatively thick transverse yarn in the backing causes a lateral gap or irregularity in the stitch spacing which cannot be in any way controlled by adjustment of the tufting machine.

Since the pile projections in a cut pile tufted fabric naturally tend to spread more effectively than in the case of an uncut pile fabric, it is, of course, feasible to tuft a lower cut pile fabric and obtain adequate coverage than is the case with an uncut or loop pile tufted fabric. The present invention permits the provision of a pile fabric having much lower pile projections, particularly in a loop pile construction, than has previously been possible and still produce a commercially saleable fabric.

In view of the above causes of unevenness in a tufted pile fabric particularly in the case of loop pile or low pile height, it might have been assumed that the use of a uniform sheet material would overcome these disadvantages. Efforts to obtain satisfactory results using a nonwoven sheet backing material have also proved fruitless because in this case there did not appear to be sufficient friction or bind on the yarns to permit uniform control of pile height, particularly after disengagement with the loopers. The precise reasons for unsatisfactory results with sheet material are not yet completely understood. It is believed that in the case of a sheet material the needle merely punches holes which do not have sufficient tendency to reclose or grip the yarns to provide adequate or at least uniform yarn engagement as the needles are removed.

In a recent patent (U.S. Pat. No. 3,110,905, issued Nov. 19, 1963 to Travis M. Rhodes) there is disclosed an improved tufted pile fabric comprising a flat woven synthetic plastic backing. For information purposes the entire disclosure of the said Rhodes patent is hereby incorporated herein by reference thereto.

Some difficulty has been encountered in attempts to commercially apply the teachings of the Rhodes patent. In particular it has been observed that tufting of the primary backings disclosed in the said patent (especially such backings woven of relatively flat cross section polypropylene yarns) causes considerable rupturing and shattering of the fill (or weft) yarns. This in turn greatly reduces the strength of the tufted pile fabric produced. The considerable strength of the yarns prior to tufting somewhat alleviates this problem. However in many instances the strength of the tufted pile fabric product is low enough to make the product commercially unacceptable. To further complicate the problem it has also been observed that the appearance of the tufted pile fabric product is frequently unsatisfactory in that the pile is uneven. This is caused by tuft-

ing needles actually breaking fill yarn ends so that tufting stitches pull through and give a product having many loops.

It is a general object of this invention to alleviate the above-described difficulties.

5 It is another object of this invention to provide synthetic plastic primary backing material adapted for use in producing high-strength tufted pile fabrics.

Another object of this invention is to provide a high-strength tufted pile fabric comprising a primary backing of 10 synthetic plastic material.

Yet another object is to provide a method for increasing the fabric strength of tufted pile fabrics comprising a primary backing of synthetic plastic material.

15 Still another object of the present invention is to provide a method for producing high-strength, high-quality tufted pile fabrics comprising a synthetic plastic primary backing material.

Many other objects, together with the numerous advantages 20 of this invention will become apparent to those skilled in the art in view of the following more detailed description.

In its broader aspects the present invention is directed to improved woven synthetic plastic primary backings treated with sufficient amounts of lubricant to provide, after tufting, a tufted pile fabric having a fabric strength of at least about 50 percent of the fabric strength of the primary backing prior to tufting. In most cases fabric strength retention is as high as 70 to 80 percent or more.

The specific amount of lubricant needed to accomplish the 30 stated objectives will vary according to the specific lubricant used, the specific primary backing to be treated, the specific type of tufting operation, etc. In general it has been found that desired results can be accomplished by treating synthetic plastic primary backing material (for example primary 35 backing materials like those disclosed in the previously mentioned Rhodes patent) prior to tufting with from about 0.2 to about 12, and preferably with about 0.6 to about 8 percent by weight, of a lubricant.

The synthetic plastic primary backings to which this invention 40 may be applied include those comprised of any of the synthetic plastic materials capable of formation into weavable yarns. Such plastics include, for example, polyethylene, polypropylene, ethylene/propylene copolymers, numerous other polymers and copolymers of other alpha olefins, 45 polyesters, polyamides, rayon, polyvinyl chloride and many other synthetic plastic materials. The invention is most especially applicable to those primary backings comprised of polypropylene yarns.

The geometry of the plastic yarns used in forming the woven 50 primary backing may be varied considerably. The invention is most efficacious with those backings in which both the warp and the fill (or weft) yarns have a relatively flat, e.g., substantially rectangular, cross section, such as those backings disclosed in the Rhodes patent previously mentioned. However,

55 significant improvements in the fabric strength of tufted fabrics comprising primary backings in which either the warp or the fill yarns (but not both at the same time) are circular or substantially round monofilament yarn and/or yarn comprised of a multiplicity of low denier monofilament (multifilament yarn). In the latter constructions it is generally preferred to utilize the round monofilament or the multifilament yarn as the fill yarns together with relatively flat cross section warp yarns. These alternate constructions, per se, do not form part 60 of the present invention and are more fully disclosed and claimed in a commonly owned U.S. application Ser. No. 487,402, filed Sept. 15, 1965, now abandoned and of which Ser. No. 885,083 filed Nov. 11, 1969 is a continuation-in-part.

The lubricant used in the practice of the present invention 70 can be any lubricating substance that does not react with, have solvent action on, or otherwise materially affect the properties of the synthetic plastic yarns in the primary backing by chemical action. Suitable exemplary materials include mineral oil; oxyethylated higher fatty acids (i.e., fatty acids having about eight carbon atoms or more) more commonly known as

polyethylene glycol esters, e.g., polyethylene glycol linoleate, polyethylene glycol stearate, polyethylene glycol oleate, polyethylene glycol laurate, oxyethylated mixtures of the fatty acids in naturally occurring higher fatty acids in various vegetable and marine oils and the like; various low molecular weight waxes, both natural and synthetic; a wide variety of well-known, nonionic surface active agents other than the oxyethylated higher fatty acids previously mentioned, e.g., those sold under the trade names Pluronic, Carbowax, etc.; and many other like materials easily recognizable to those skilled in the art. Preferably the lubricant should be a relatively low-viscosity liquid either as such or when in water emulsion, so as to provide easy application and spreading. The most especially preferred lubricants (based on experimental results to date) are mineral oil and the polyethylene glycol oleate (having an average of about 15 oxyethylene ( $-\text{CH}_2\text{CH}_2\text{O}-$ ) groups per molecule) commercially sold under the trade name Nopcostat 2152-P.

Treatment of the synthetic plastic primary backing material with the desired lubricant can be accomplished in a variety of ways. It is for example permissible to treat either the respective warp or fill yarns or both warp and fill yarns with the lubricant prior to weaving them to form the backing. It will be clear that lubricant treatment can take place after the primary backing material is woven but before it is tufted. This may or may not be a preferred procedure depending upon the particular plant in question i.e., whether weaving and tufting are performed in-line or in the same plant facilities and whether the weaver or tufter is capable of or willing to become capable of performing the lubricant treatment.

In a presently preferred embodiment the lubricant treatment required for the practice of the present invention is ac-

10 been woven experience to date has indicated that treatment can range from about 1 to about 12 and preferably from about 2 to about 8 percent by weight of lubricant based on the total weight of the primary backing. It will be noted therefore, that lubricant treatment of fill yarn alone can result in some savings in the amount of lubricant needed.

15 Regardless of the point in time of the lubricant treatment, it can be readily accomplished by spraying, dipping, roll coating, or otherwise applying the lubricant or a solution (provided that the solvent has no action on the plastic yarns) or emulsion containing the same to the plastic yarn prior to weaving, or to the primary backing after it is woven.

The invention is illustrated in the following nonlimiting examples.

#### EXAMPLE 1

A primary backing was woven from polypropylene ribbon yarns in a conventional pattern of 15 warp yarns and 10 fill 20 yarns per inch on a laboratory scale to produce a backing 1 yard wide. The warp yarns were not lubricated. The fill yarns were lubricated the maximum possible extent by hand drawing through a bath of polyethylene glycol oleate lubricant (Nopcostat 2152-p), giving lubricant treatment far in excess of that normally occurring in conventional yarn processing. The heavily lubricated fill yarn was quilled on a conventional Whitin quiller, over end. For comparison unlubricated fill 25 yarns were woven in identical manner into primary backings.

Each of the primary backings thus prepared was tufted on a laboratory scale 14-inch wide tufted using 10 stitches per inch and 6.5 rows per inch of 3700 denier Type 501 nylon and  $\frac{1}{4}$  inch pile height. Results are summarized in the following table I.

TABLE I

| Run | Warp and fill yarn                                                             | Fill yarn lubrication | Average fabric fill strength <sup>1</sup> |        | Average fabric warp strength <sup>1</sup> |        |
|-----|--------------------------------------------------------------------------------|-----------------------|-------------------------------------------|--------|-------------------------------------------|--------|
|     |                                                                                |                       | Untufted                                  | Tufted | Untufted                                  | Tufted |
| 1   | 1080 denier polypropylene ribbon<br>100 mils wide,                             | None                  | 84                                        | 27     | 200                                       | 155    |
| 2   | do                                                                             | Yes                   | 84                                        | 74     | 179                                       | 183    |
| 3   | Same as 1 for warp; 1080 denier polypropylene ribbon, 130 mils wide, for fill, | None                  | 104                                       | 25     | >200                                      | 140    |
| 4   | do                                                                             | Yes                   | 100                                       | 58     | 192                                       | 165    |

<sup>1</sup> Determined on Instron tensile tester using a 4 by 6 inch test sample (6 inches in test direction), a distance of 3 inches between jaws, a 12 inch per minute constant jaw travel rate and jaws 1 inch wide and  $1\frac{1}{2}$  inches long. Care is taken in placing samples in jaws to be sure that the same individual yarns are gripped by the respective jaws. The results are reported in pounds required to break per fabric inch (lbs./inch). The values shown are average of 4 separate tests on fill direction samples and 3 tests on warp direction samples.

complished by excessively lubricating the warp yarns prior to placing them on the loom beam used in the weaving operation. This essentially eliminates the need for lubricating the fill 50 yarns. It is to be understood, however, that lubrication of the fill yarns alone will also accomplish the desired results.

As indicated previously, the invention is broadly directed to lubricant treatment sufficient to provide 50 percent or more fabric strength retention in tufted pile fabrics utilizing synthetic plastic primary backings. The basic purpose of the lubricant treatment is to deter physical damage to the fill yarns by the tufting needles in the tufting machine. This could perhaps be accomplished by lubricating the needles themselves but this is believed to be impractical for the tufted.

As indicated above lubrication of the fill yarns alone will satisfy the purposes of this invention. Present experience indicates that treatment of fill yarns with from about 0.5 to about 10 percent by weight, and preferably about 1.5 to about 7 percent, based on the yarn weight, together with no lubricant treatment of the warp yarns, gives quite satisfactory results. Inasmuch as the fill yarns comprise about 40 percent of the total primary backing the filling yarn treatments stated correspond approximately to about 0.2 to about 4 (preferably about 0.6 to about 3) percent by weight of lubricant, based on the weight of the total backing.

When treating both the warp yarns and the fill yarns before weaving, or when treating warp yarns alone before weaving, or when treating the synthetic plastic primary backing after it has

60

55

65

70

75

50 The striking differences in fabric strength retention after tufting, particularly in the fill direction, are readily apparent from the data of table I.

In addition it was observed that tufted appearance was grossly different. Both lubricated samples (Runs 2 and 4) had good pile evenness. The unlubricated controls (Runs 1 and 3), representing known primary backings, each had many loops caused by tufting needles actually breaking filling ends so that tufting stitches pulled through.

#### EXAMPLE 2

A polypropylene yarn primary backing identical to that of Run number 2 of example 1 was prepared and tufted by a commercial carpet manufacturer in a zigzag,  $7\frac{1}{2}$  stitches per inch and  $6\frac{1}{2}$  rows per inch. Average fabric strengths, in the fill direction, determined as described in footnote 1, table 1 were:

Untufted—93 pounds per fabric inch

Tufted—70 pounds per fabric inch

For comparison a commercially available woven jute primary backing (16 warp yarns per inch and 13 fill yarns per inch) was tufted in an identical manner. Average fabric fill strengths were:

Untufted—71 pounds per linear inch

Tufted—25 pounds per linear inch

## Example 3

A polypropylene yarn primary backing identical to that of Run number 4 of example 1 was prepared and tufted by a commercial carpet manufacturer 9½ stitches per inch, 9½ rows per inch with a cut pile one-fourth inch high after which the tufted pile fabric was piece dyed. Average fabric strength (3 samples) in the fill direction after tufting and dyeing was 82 pounds per fabric inch. All samples tested in the warp direction gave fabric strength results greater than 200 pounds per inch.

## EXAMPLE 4

In this example further polypropylene ribbon primary backings substantially like those in Runs 1 and 2 of example 1 were prepared. The backings of this example were woven 12 feet wide on a commercial loom using a Unifil quiller with no lubricant applied to the fill yarns. The warp yarns were very heavily lubricated with Napcostat 2152-P prior to placement on the loom beam used in the weaving operation. Paired samples of the primary backings so prepared were tufted with and without preliminary heat setting of the backing on a tenter frame. Tufting was substantially identical to that used in example 1, the only difference being tufts at 9½ stitches per inch instead of 10 stitches per inch. In addition still further backing samples were tufted at 6½ stitches per inch with no preliminary heat setting of the backing. Results are summarized in table II. The average fabric strengths were determined as described in example 1 except that untufted strengths represent an average of three instead of four readings.

TABLE II

| Run No.: | Average fabric strength (fill direction) |              |          |                      |        |
|----------|------------------------------------------|--------------|----------|----------------------|--------|
|          | Tufted, 9½ stitches per inch             |              |          |                      |        |
|          | Untufted                                 | Not heat set | Heat set | 6½ stitches per inch | Tufted |
| a-----   | 99                                       | 79           | 84       | 78                   |        |
| b-----   | 100                                      | 76           | 80       | 76                   |        |

When samples were woven and tufted in exactly the same manner except for lubricant treatment of the fill yarn in addition to the very heavy treatment of the warp yarns results were as follows:

TABLE II A

| Run No.: | 98 | 84 | 84 | 78 |
|----------|----|----|----|----|
| c-----   | 91 | 84 | 82 | 82 |

<sup>1</sup> The difference between runs c and d was the use of a different lubricant and lubricant concentration. Both lubricants used are commercially available materials.

The results shown in tables II and II A show that lubricant treatment of the fill yarns is not needed to get good tufted fabric strength when the warp yarn is very heavily lubricated prior to weaving. This is a highly significant advantage in view of the difficulties sometimes experienced in quill weaving with highly lubricated fill yarns.

The results further show that heat setting (1 minute at 280° F.) had little or no significant effect on tufted fabric strength.

## EXAMPLE 5

This example illustrates the use of the invention with primary backings having substantially flat warp yarns (15 ends per inch) like those of used in example 1, Run 1 and circular or round monofilament or multifilament fill yarns. In all instances the yarns used were comprised of polypropylene. The backings contained 8 ends per inch of round monofilament fill yarn and 10 ends per inch of multifilament fill yarn. The fill yarns were lubricated prior to weaving with mineral oil or

commercially available polyethylene glycol oleate (Nopcostat 2152-P). The strength retention values presented are calculated from the formula:

$$5 \quad \text{Percent Strength retention} = 100 \frac{\text{Yarn tensile strength after weaving and Tufting}}{\text{Initial tensile strength of yarn}}$$

Results are summarized as follows:

| Fill Yarn Description                                        | Strength Retention |
|--------------------------------------------------------------|--------------------|
| 960 denier round monofilament                                | 91%                |
| 800 denier round monofilament                                | 91%                |
| 700 denier round monofilament                                | 84%                |
| 15 1,120 denier multifilament<br>(16 threads—70 denier each) | 78%                |
| 1,200 denier multifilament<br>(8 threads—150 denier each)    | 100%               |

20 As previously noted the above structures, per se, are more fully disclosed and claimed in commonly owned U.S. application Ser. No. 487,402 filed Sept. 15, 1965, now abandoned, of which application Ser. No. 884,083 filed Dec. 11, 1969 is a continuation-in-part.

25 Variations and modifications of the instant invention will become apparent to those skilled in the art upon reading the foregoing description and illustrative examples. All such variations and modifications are considered to be within the scope of the appended claims.

30 Many advantages of the present invention have been fully described and illustrated hereinabove. It is also expected that the invention will result in a substantial increase in tufting efficiency in commercial operations with little or no additional cost to the commercial tufter. In particular there surely will be 35 less wastage (in view of the greatly improved tufted pile appearance). Moreover, substantially less down time because of tufting yarn breakage is expected in view of increased ease of tufting and resultant decreased strain on tufting yarn in the tufting needles.

40 I claim:

1. A high-strength tufted pile fabric comprising a woven primary backing material, said primary backing woven of yarn of a plastic selected from the group consisting of polypropylene and copolymers of propylene, at least some of said yarn in said primary backing having a relatively flat cross section; said substantially flat yarn being coated with a lubricant in an amount in the range of about 0.2 to 12 percent based on the weight of said yarn, and a plurality of tuft, a substantial number of said tufts penetrating some of said lubricated substantially flat yarn, said penetrated yarn being relatively free of ruptured and shattered areas compared to an unlubricated penetrated yarn in otherwise similar fabric.

2. A high-strength tufted pile fabric comprising a woven primary backing material, said primary backing woven of yarn made from a polymer selected from the group consisting of polypropylene and copolymers of propylene, at least some of said yarn in said primary backing having a substantially flat cross section, said substantially flat yarn coated with an agent that is essentially nonreactive with and having essentially no solvent action on said yarn, said agent being present in an amount of about 0.6 to 8 percent based on the weight of said yarn, said agent being selected from the group consisting of mineral oil and oxyethylated higher fatty acids, and a plurality of tufts, a substantial number of said tufts being inserted 55 through said woven primary backing with a frequency of more than 6½ tufts per inch, some of said tufts that are inserted with a frequency of more than 6½ tufts per inch penetrating some of said lubricated substantially flat yarn, said penetrated yarn being relatively free of ruptured and shattered areas, said 60 high-strength tufted pile fabric having a fabric strength in the fill direction of at least 50 pounds per linear inch.

UNITED STATES PATENT OFFICE  
CERTIFICATE OF CORRECTION

Patent No. 3,613,612 Dated October 19, 1971

Inventor(s) Carroll Trowbridge Kennedy.

It is certified that error appears in the above-identified patent and that said Letters Patent are hereby corrected as shown below:

Column 2, line 68, cancel "Ser. No. 885,083 filed

Nov. 11, 1969" and insert --Ser. No. 884,083 filed

Dec. 11, 1969--;

Column 6, line 46, cancel "year" and insert --yarn--;

line 48, cancel "tuft" and insert --tufts--.

Signed and sealed this 19th day of December 1972.

(SEAL)

Attest:

EDWARD M.FLETCHER, JR.  
Attesting Officer

ROBERT GOTTSCHALK  
Commissioner of Patents